

1

2,842,510

## QUEOUS FIREPROOFING COMPOSITION OF SODIUM OXYFLUOBORATE AND PHENOL FORMALDEHYDE, METHOD OF TREATING PAPER THEREWITH AND ARTICLE PREPARED THEREFROM

James A. Robertson, Lewiston, N. Y., assignor to E. I. du Pont de Nemours and Company, Wilmington, Del., a corporation of Delaware

No Drawing. Application August 15, 1955  
Serial No. 528,561

7 Claims. (Cl. 260—29.3)

This invention relates to flame-resistant paper. More particularly, it relates to paper made flame-resistant in such a manner that it is no stiffer than paper not flame-resistant.

In U. S. Patent 2,823,145, issued February 11, 1958, there is revealed a new and excellent method of fireproofing inflammable materials, cellulosic fibers in particular. This method consists in supplying to the fibers an oxyfluoborate of the formula  $NaF \cdot xB_2O_3$  where  $x$  varies between about 1.17 and 1.45, or a hydrate thereof. Especially valuable is the compound  $NaF \cdot 1.25B_2O_3$  and its hydrates. These compounds and methods for their preparation are claimed in U. S. Patent 2,823,095, also issued February 11, 1958.

While the oxyfluoborates afford very good flameproofing to cellulosic bases, they suffer from the disadvantages of stiffening the material to which they are applied. The stiffening action is thus noticeable when the compounds are applied to converted paper products or cardboard also containing a modifying agent. Paper impregnated with a modifying agent such as a water-soluble phenol-formaldehyde mixture is frequently prepared for sale to customers who shape the paper as desired and heat the same to cure the resin. The shape is set permanently in the base by this treatment. When oxyfluoborates are added to paper simultaneously with the phenol-formaldehyde and the paper is dried, it may become so stiff that it cannot be bent readily and uniformly. Use of oxyfluoborates as fireproofing agents in paper containing thermosetting monomers has thus, heretofore, been somewhat inconvenient.

An object of this invention is, consequently, provision of paper or other fibrous articles containing both oxyfluoborates and the uncured form of thermosetting resins, phenol-formaldehyde in particular, which are not too stiff to be bent readily.

Another object is provision of a method for supplying both oxyfluoborates and thermosetting resins to a paper base without stiffening the base excessively when the latter is dried.

The above-mentioned and still further objects are achieved in accordance with this invention by impregnating inflammable bases, paper in particular, from an aqueous solution containing the uncured form of the thermosetting resin, an oxyfluoborate and also a plasticizer of the group consisting of water-soluble polyhydric alcohols and water-soluble polyethylene glycols. These plasticizing agents are not operative to soften paper impregnated with oxyfluoborates alone. Their effect in their present usage is thus quite surprising.

The oxyfluoborates of the impregnating solution are, of course, those of U. S. Patent 2,823,145. A preferred composition is  $4NaF \cdot 5B_2O_3$  or the hydrate



The quantity of oxyfluoborate dissolved is determined basically by the percentage of flameproofing agentulti-

2

mately desired in the paper. This percentage is generally between about 5 and 15% by weight. Since there is no preferential absorption with the oxyfluoborates, or with any other material used in the present solution, the percentage of compound (hydrate) in solution should be about the same, i. e., 5-15% by weight. This statement is based on the approximately correct assumption that there is 100% absorption from solution.

The preferred thermosetting resin for use in the paper of this invention is phenol-formaldehyde. Consequently, the precursor of this material, A stage phenol-formaldehyde, is also included in the impregnating solution. The quantity of this material dissolved is also determined ultimately by that needed in the paper product. About 11-13% by weight is generally used in the paper but smaller quantities are acceptable. To insure that the desired quantity is absorbed from the solution, about 15% by weight of the solution should consist of the A stage material. Between about 5 and 15% by weight is usually satisfactory and will deposit roughly about 5-15% by weight of the paper on the paper when the latter is wetted with its own weight of solution. Other thermosetting resins besides phenol-formaldehyde may be employed in this process. These include urea-formaldehyde, melamine-formaldehyde and the like. The quantity of these materials necessary is roughly equivalent to that of phenol-formaldehyde, both in solution in the A stage form and on the paper, ultimately, as the polymer.

The preferred polyhydric alcohols for use to soften paper impregnated with the organic monomers and oxyfluoborate are glycerine and ethylene glycol but others may be used as well. The quantity employed will vary with the combined weight of flameproofing agent and monomers and, in the case of glycerine, may comprise up to about 15% by weight of this weight. About 5% is preferred, based upon the weight of oxyfluoborate hydrate either in solution or on the dried paper. Above 5% can be used but the higher percentages yield no commensurate gains and hence are not desired.

The water-soluble polyethylene glycols having molecular weights between about 200 and 20,000 are suitable for the purposes of the invention. A molecular weight of about 1500 gives the best results. The quantity of these polyglycols required is about the same as that of the polyhydric alcohols. Thus between about 5 and 15% by weight, based on the weight of the oxyfluoborates, is preferred.

Polyethylene glycols are conveniently supplied to the impregnating solution as "Carbowax." This is the trade name of glycols sold by the Carbide and Carbon Chemicals Corporation and is defined in the *Handbook of Material Trade Names*, Zimmerman and Lavine, Industrial Research Service (1953). The molecular weight of the polyglycol is determined by the number affixed to "Carbowax." Thus "Carbowax" 1500 has a molecular weight of 1500.

One factor which influences to some extent the chosen concentration of all agents in the solution is the contact time between it and the untreated paper. The values given are effective for about the minimum time required for thorough wetting of paper normally encountered in commerce. At thorough wetting the paper absorbs about 100% of its weight of solution. When the water is evaporated, the percentage of solid deposited will be slightly less than the percentage in solution. Thorough wetting occurs in a matter of seconds, for ordinary paper being essentially the time required to dip the paper slowly into solution and remove it. Greater solution concentrations may be employed if very rapid dips are required. Adjustment of solution concentration

and contact time to obtain a particular concentration of solids on the paper is, in any case, very simple where there is no preferential absorption. Room temperature, i. e., 20-25° C., is effective for this contact but higher temperatures may be employed.

The composition of the aqueous impregnating solutions may now be summarized. To obtain a flame-resistant paper soft enough for convenient manipulation but containing sufficient A stage material for ultimate strength, the aqueous solution may comprise about 5-15% by weight of the oxyfluoborate hydrate, about 5-15% by weight of phenol-formaldehyde, and 0.5-1.5% by weight of glycerine or other water-soluble polyhydric alcohol. Such a solution will yield a dried paper containing about 5-15% of the flame-resistant agent, about 5-15% of the thermosetting material and 0.5-1.5% of the plasticizer, again assuming 100% absorption from solution. When the polyethylene glycols are substituted for the polyhydric alcohols, about 0.5-1.5% of the former is included in solution to yield a paper containing the same quantity of plasticizer.

The process may also be summarized. Paper is dipped into a solution of one of the compositions given above at room temperature for about the minimal time complete wetting. The paper is then removed and dried as convenient. It will be understood that the drying temperature is less than that needed to set the resin. The steps enumerated so far are those of a primary manufacturer and yield an intermediate product to be operated upon by secondary manufacturers. The steps taken by the latter are (1) forming the basic paper product into any desired shape and (2) heating the shape to cure the thermosetting resin. These final steps yield a product retaining its shape indefinitely.

"Stiffness" or "softness" as used in this application is not qualitative. It can, on the contrary, be measured quantitatively as on a Tinius-Olsen stiffness tester. This is an instrument sold by the Tinius-Olsen Company of Philadelphia, Pennsylvania. Results are expressed in arbitrary units proportional to the resistant force exerted by the paper or other material as it is twisted through various angles.

There follow some examples which illustrate the invention in detail. In these examples all percentages are

given in terms of weight. Stiffness tests were made at room temperature on the Tinius-Olsen tester mentioned above.

A series of experiments was carried out in which ordinary heavy kraft wrapping paper was dipped at room temperature into solutions containing various impregnants, dried and tested for stiffness. Results and other pertinent data are given in the table. In the table OFB is  $4\text{NaF}\cdot 5\text{B}_2\text{O}_3\cdot 5\text{H}_2\text{O}$ , PF is phenol-formaldehyde in the common "A-stage" form, G is glycerine, C2 is "Carbowax" 200, C3 is "Carbowax" 1500, C6 is "Carbowax" 6,000 and C20 is "Carbowax" 20,000.

Having described my invention, I claim:

1. An aqueous solution for fireproofing paper and other fibrous articles which comprises about 5-15% by weight of sodium oxyfluoborate hydrate, about 5-15% by weight of A stage phenol-formaldehyde and about 0.5-1.5% by weight of a water-soluble softening agent of the group consisting of glycerine, ethylene glycol, and polyethylene glycols having a molecular weight between about 200 and 20,000.
- 15 2. An aqueous solution for flameproofing paper and other fibrous articles which comprises about 5-15% by weight of sodium oxyfluoborate hydrate, about 5-15% by weight of A stage phenol-formaldehyde and about 0.5-1.5% by weight of glycerine.
- 25 3. An aqueous solution for flameproofing paper and other fibrous articles which comprises about 5-15% by weight of sodium oxyfluoborate hydrate, about 5-15% by weight of A stage phenol-formaldehyde and about 0.5-1.5% by weight of a water-soluble polyethylene glycol having a molecular weight between about 200 and 20,000.
- 30 4. The method of producing paper which is soft and yet fireproofed by means of sodium oxyfluoborate which comprises immersing the paper to be treated for a short time in an aqueous solution comprising about 5-15% by weight of sodium oxyfluoborate hydrate, about 5-15% by weight of A stage phenol-formaldehyde and about 0.5-1.5% by weight of a water-soluble softening agent of the group consisting of glycerine, ethylene glycol, and polyethylene glycols having a molecular weight between about 200 and 20,000, and subsequently drying the treated paper at a temperature less than that required to set the resin.
- 35 5. The article produced by the method of claim 4.
- 50 6. The method of producing a fireproofed, shaped article which comprises immersing paper for a short time in an aqueous solution comprising about 5-15% by weight of sodium oxyfluoborate hydrate, about 5-15% by weight of A stage phenol-formaldehyde and about 0.5-1.5% by weight of a water-soluble softening agent of the group consisting of glycerine, ethylene glycol, and polyethylene glycols having a molecular weight between about 200 and 20,000, drying the treated paper, forming the paper into the desired shape and heat-curing the shape to produce thermoset phenol-formaldehyde, and thereby permanently setting the shape in the paper.
- 55 7. The article produced by the method of claim 6.

#### References Cited in the file of this patent

#### UNITED STATES PATENTS

- 2,594,280 Beaudet \_\_\_\_\_ Apr. 29, 1952  
 2,639,242 Suen \_\_\_\_\_ May 19, 1953

#### OTHER REFERENCES

- Ryss et al.: "Chem. Abstracts," volume 48 (July 25, 1954), edition 8014b.

<sup>1</sup> Absorption from solutions was somewhat less than 100%. The percentage of dissolved material in the impregnating solution was 18%.